

# United States Patent

McCard

[15] 3,696,601

[45] \*Oct. 10, 1972

[54] TEXTILE HEATING AND COOLING

[72] Inventor: Henry W. McCard, 208 Rodman Avenue, Jenkintown, Pa. 19046

[\*] Notice: The portion of the term of this patent subsequent to July 7, 1987, has been disclaimed.

[22] Filed: Nov. 7, 1969

[21] Appl. No.: 874,764

Related U.S. Application Data

[63] Continuation-in-part of Ser. No. 751,785, Aug. 12, 1968, Pat. No. 3,518,822.

[52] U.S. Cl. .... 57/34 HS, 34/23, 34/155, 34/160, 57/157 TS

[51] Int. Cl. .... D02g 1/02

[58] Field of Search.... 34/23, 155, 160; 57/34 HS, 57/157 TS; 28/62

[56] References Cited

UNITED STATES PATENTS

|           |         |                |          |
|-----------|---------|----------------|----------|
| 2,316,984 | 4/1943  | Brockel .....  | 34/155 X |
| 2,509,279 | 5/1950  | Sisson .....   | 34/23 X  |
| 2,657,433 | 11/1953 | Merriman ..... | 34/23 X  |
| 2,943,433 | 7/1960  | Van Dijk ..... | 57/34 HS |

|           |         |                             |
|-----------|---------|-----------------------------|
| 3,091,908 | 6/1963  | Carruthers..... 57/34 HS    |
| 3,237,392 | 3/1966  | Crouzet..... 57/34 HS       |
| 3,368,335 | 2/1968  | Horvath..... 57/34 HS       |
| 3,411,282 | 11/1968 | Hampel..... 57/34 HS        |
| 3,420,983 | 1/1969  | McCard et al. .... 28/62 X  |
| 3,461,657 | 8/1969  | Scragg et al. .... 57/34 HS |
| 3,518,822 | 7/1970  | McCard..... 57/34 HS        |

Primary Examiner—John Petrakes  
Attorney—Jackson, Jackson & Chovanes

[57] ABSTRACT

In order to accomplish rapid cooling of synthetic thermoplastic continuous filament yarn which has been heated for bulking or the like, the yarn is led along a groove and subjected to jets of cooling gas spaced along the groove. For bulking in the preferred form the yarn is false twisted and heated suitably by a rotating drum heater having a smooth descending conical portion toward a take off end, and a downward step at one end of the smooth conical portion. In another form, the drum heater has two right cylindrical portions of different diameter, the smaller being at the outlet end, and a step separating them. In another form two ends of yarn are applied, and then the yarn is continuously brought into or against a heater, preferably a rotating drum heater.

9 Claims, 8 Drawing Figures



PATENTED OCT 10 1972

3,696,601

SHEET 1 OF 3



INVENTOR

Henry W. McCord

BY

Jackson, Jackson and Kovacev

ATTORNEYS

PATENTED OCT 10 1972

3,696,601

SHEET 2 OF 3



Fig. 2



Fig. 8.



Fig. 7.

INVENTOR.

Henry W. McCord

BY  
Jackson, Jackson and Clowes

ATTORNEYS.

PATENTED OCT 10 1972

3,696,601

SHEET 3 OF 3



## TEXTILE HEATING AND COOLING

The present application is a continuation-in-part of my copending application Ser. No. 751,785, filed Aug. 12, 1968, for Textile Heater and Process, now U.S. Pat. 3,518,822.

## DESCRIPTION OF INVENTION

The present invention relates to textile machinery for producing bulked synthetic thermoplastic continuous filament yarn and to processes therefor.

A purpose of the invention is to improve the rapid cooling of synthetic thermoplastic continuous filament yarn which has been heated in order to permit it to shrink and bulk and particularly to render cooling possible at higher speeds of yarn progression.

A further purpose is to false twist yarn, to heat the false twisted yarn, preferably by a rotating drum heater to be described, and to cool the yarn by cooling gas jets against its side along a groove.

A further purpose is to ply two ends of synthetic thermoplastic continuous filament yarn twisted with respect to one another, to bring the plied yarn against the outside of a rotatable drum heater so as to heat the yarn and to drop the yarn over a step at one end or the other of the smooth conical portion, and then cool the yarn by progressing it in airborne fashion along a groove where it is subjected to a series of transverse cooling gas jets, and finally to separate the yarn ends.

A further purpose is to heat the yarn to be false twisted by a drum having a large inlet right cylindrical portion and a small outlet right cylindrical portion separated by a step, the small portion preferably having groove walls separating yarn paths.

Further purposes appear in the specification and in the claims. FIG. 1 is a diagram showing the complete textile operation of plying two yarn ends twisted together, heating on a drum heater, rapidly cooling to set the bulk effect and then deploying or separating the yarn ends and forming packages.

FIG. 2 is a diagram showing bulking of yarn by false twisting according to the preferred form of the invention.

FIG. 3 is a fragmentary axial section of a preferred drum heater according to the invention.

FIG. 4 is a perspective of the cooling mechanism illustrated, with a portion broken away to show the construction at the cooling groove.

FIG. 5 is a section of one form of cooling mechanism on the line 4—4 of FIG. 3.

FIG. 6 is a diagrammatic cross-sectional illustration of the yarn traveling along the groove.

FIG. 7 is a fragmentary side elevation of the cooling device showing a preferred orientation of the orifices.

FIG. 8 is a side elevation a further variant form of heater drum of the invention.

In the prior art numerous processes have been developed for creating bulk and yarn stretch characteristics in synthetic thermoplastic continuous filament yarn such as nylon and the like. The problem is rendered difficult by operation at higher and higher linear speeds, speeds of 40 yards per minute now being employed, and spindle speeds sometimes running as high as 150,000 rpm.

Usually the creation of bulk and stretch characteristics involves a combination of heating and twisting and then cooling so that the effect of the twist is set.

While strip heaters have been used, there is a considerable advantage in employing rotatable drum heaters, for example, according to McCard and Ross U.S. Pat. No. 3,420,983, granted Jan. 7, 1969, for 5 Rotating Drum Heater for Synthetic Yarn.

In a preferred embodiment of the invention, synthetic thermoplastic continuous filament yarn is run through a false twister. While the yarn is subjected to false twist it is heated preferably by a drum heater to be described, or by a strip or other heater. While the heated yarn is still subjected to twist and heat, it is suddenly cooled by running along a groove past cooling gas jets.

When false twist is applied to yarn heated on some drum heaters, the yarn undergoes shrinkage as a result of the heating and cooling, and there is a pronounced tendency, even if the heater allows for the shrinkage, for the yarn ends to break at or adjacent to the drum heater. In my U.S. Pat. Application Ser. No. 751,785, above referred to, provision has been made to correct this difficulty. The breakage is due to the tendency of false twist to back up toward the place from which the yarn is coming.

25 By bringing untwisted yarn on to the heater drum on a smooth cylindrical pre-heating section and then passing the yarn along a smooth conical portion having an abrupt step at one or the other end thereof, allowance is made for backing up of the twist from the spindle to and on to the heater drum. Yarn ends tend to adjust their position along the axis of the drum to compensate for the backup of the twist.

30 In another form of drum configuration, which I have found to be satisfactory for processing false twist yarn, the yarn is brought on to the smooth cylindrical pre-heating section of the drum and is led over the separator pin and then on to the drum repeatedly, until a sufficient number of passes have been made so the contact time at temperature is sufficient to raise the yarn to its 35 plastic temperature range. The yarn is then led into the grooves (all of the same diameter, approximately) which permits the twist to back up on to the heated drum and to be heated and heat-set in the twisted state.

40 One of the difficulties still remaining is that it is important to accomplish the cooling very quickly, notwithstanding the rapid forward progression of the yarn which has been heated. If the cooling is accomplished by direct surface contact, there is danger of creating 45 stress in the yarn in contact with the cooling surface, and abrading the yarn against such surface. One of the 50 important features of the present invention is to support the yarn in an airborne condition as it is subjected to cooling gas, preferably air. Reliance is had on Bernoulli's principle to keep the yarn airborne as it is subjected to a sequence of transverse gas jets.

55 One way of false twisting the yarn of the invention is by the duo-twist process which is used for creating bulk and stretch by twisting two yarn ends together to 60 produce plied yarn to render it thermoplastic and then cooling to set the yarn, the bulked yarn ends being subsequently separated and formed into packages. See Carothers U.S. Pat. No. 3,091,908, granted June 4, 1963.

65 It is believed that the best application of the invention is likely to be in creating nylon yarn with bulked and stretch characteristics from nylon continuous fila-

ment yarn usually having multifilaments. For this purpose, the outside temperature of the heating drum should be approximately 400° F., that is, in the range between 350° and 450° F., which will render the nylon thermoplastic.

The invention is also applicable to other continuous filament synthetic thermoplastic yarns at appropriate temperatures for heating each of them, for example polyester, polyvinylchloride, polyvinylchloride acetate and polypropylene yarns.

The invention is intended to be applied to continuous filament synthetic thermoplastic yarn, examples being 70 denier, 34 filament nylon yarn, and 17 denier, 17 filament nylon yarn.

The broad concept of running yarn over a cone with takeoff at the small end is old in Cadden U.S. Pat. No. 2,218,504, granted Oct. 22, 1940, and Stanley U.S. Pat. No. 3,221,385, granted Dec. 7, 1965. Running yarn over a cone with takeoff at the large end is shown by Cotchett U.S. Pat. No. 2,174,688, granted Oct. 3, 1939, and McCrosky U.S. Pat. No. 2,370,180, granted Feb. 27, 1945. None of these devices provides a cylindrical drum heater having a smooth cone descending from the cylinder to a takeoff at the small end with an abrupt step at one or the other end of the smooth conical portion.

FIG. 1 illustrates diagrammatically equipment to which the invention is applicable, and a process for creating bulked thermoplastic continuous filament yarn. This Figure shows a duo-twist installation for creating bulked and stretch characteristics in continuous filament thermoplastic yarn, such as nylon.

A yarn end 20 is withdrawn from a source of yarn 21 and passes through the hollow interior of a stationary bobbin 22 supported at a point 23 near its upper end. Another synthetic continuous filament thermoplastic yarn end 24 is withdrawn from a source 25 and wrapped in a series of helical turns 26 around the outside of the bobbin 22, the wrapping being accomplished in any suitable manner, not shown. Turns of the yarn end 24 are progressively formed at the upper end and withdrawn at the lower end of the bobbin so that at point 27 each of the yarn ends 20 and 24 is plied together, being helically wound one with respect to the other, as well known in the art.

The two-ply thermoplastic yarn 28 is brought into tangential contact with the outside of a suitably metallic heater drum 30 shown more in detail in FIG. 3 and specifically forming the subject matter of my U.S. Pat. application Ser. No. 751,785 above referred to. The yarn enters the heater drum 30 at its inlet end 31 and progresses along the outside of the drum to the takeoff end 32.

At the inlet end 31 the yarn encounters a straight outside right cylindrical portion 33 which is of short extent since its main function is to preheat the yarn as it passes around the cylindrical portion. Then in the form of FIGS. 1 and 3, the yarn encounters an abrupt descending step 34 which is placed approximately at the point where extensive shrinkage occurs (nylon continuous filament undergoes 14 percent shrinkage in the thermoplastic range). A step dimension of 0.05 inch on a side has been found to be adequate. Then follows a smooth gradual descending conical portion 35 to the takeoff end 32. While various angles may be used on

this descending conical portion, depending on the extent of backup of twist to be compensated for, the angle of the conical portion should preferably be in the range from about 5° to 25°, and more desirably about 15° with respect to the axis of the drum.

Around the conical portion 35 of the drum there will suitably be from three to five or six loops of yarn 38, each of which passes around the outside of a guidepost 37 which is positioned adjoining and off to one side of the drum. The guidepost 37 may be stationary or it optionally may rotate like a spool if desired, as shown in my copending application above referred to.

The post 37 has guide grooves at the ends to retain the yarn.

A rim 40 at the inlet end prevents the yarn from running off the drum at that end, and rim 41 at the takeoff end prevents the possibility that the yarn will run off the drum at that end, and rim 41 at the takeoff end prevents the possibility that the yarn will run off the drum at that end.

In many installations the drum heater will provide all the heat that is necessary, but in FIG. 1 I show an optional supplemental longitudinal or strip heater 42 having a heating chamber 43 through which the plied yarn 28 passes.

From the last heater, the plied yarn is guided over canted rolls 44 and 45 so that it cools while twisted to begin the cooling operation. Then the yarn passes along a cooling groove 46 of a yarn cooler 47 best seen in FIGS. 4, 5, and 6. The groove is wide enough to admit the yarn with space on either side as best seen in FIG. 6.

Distributed along the length of the groove at the back is a plurality of transverse nozzles 48 which discharge a cooling gas, suitably air, from a plenum chamber 50 connected to a source, suitably compressed air, by a connection 51. Using nylon yarn of the character discussed above, with a cooling groove having a depth of 0.010 inch and a width of about one-eighth inch, nozzles about 0.034 inch in diameter every half inch have proved to be adequate with air pressure supplied from the plenum chamber in a range which may vary between 5 and 30 psi. The yarn passing along the groove tends to float or become airborne as shown in FIG. 6, and to center itself with respect to the groove because of Bernoulli's principle, thus being cooled without the danger of abrasion which might occur if the yarn were following the outside surface of a metallic cooling element at this time. It should be remembered that rapid cooling is a very critical operation because the yarn tends to shrink very rapidly.

After cooling, the plied ends are separated into bulked yarn ends 52 and 53 which pass through guides 54 and 55 to form packages 56 and 57.

Thus the synthetic thermoplastic continuous filament yarn ends 20 and 24 are first plied together and helically wound around one another and then heat set and rapidly cooled and deplied to form bulked and stretch-capable yarn ends 52 and 53. Yarn of this character is believed to be of special value to produce the panty portion of ladies' stocking-and-panty combinations.

As the heater drum operates in FIG. 1, the tension on the individual turn may vary and rather than breaking the loops, readjustment is likely to take place by slipping of the loops along the conical portions or fail-

ing to slip along the conical portions of the drum heater and by pulling of loops from the cylindrical portion of the drum over the step. This effect varies with the extent to which twist backs up onto the conical portion of the drum as a result of the twist introduced and of the deplying action which separates the bulked ends. An equilibrium condition is reached between the tendency of the twist to back up onto the cone and the tendency of the loops to slip down the cone, and thus the machine operates effectively at high speed without serious breakage.

The drum 30, as shown in FIG. 3, has a hollow interior 58 so that it can surround a heater. A suitably hollow shaft 60 is journaled on antifriction bearings 61 mounted in a housing 62, and at the outer end provided with a flange 63. The shaft has an opening 64 which permits air to circulate to cool the bearings. At the outer end of the shaft 60 there is provided a conical portion 65 which seats in a central conical opening 66 on the drum and is held in place by a screw 67 threaded into the end of the shaft. Depending on the installation, the drum may idle under the forward motion imparted by the takeup mechanism to the yarn by means not shown, or the shaft may be driven, suitably by a drive which has limited torque capability, such as a shaded pole electric motor so that the drum speed will respond to variations in the tendency of the yarn to move forward.

Within the hollow of the drum there is placed a heater 68. While the heater can operate on steam, hot air or other suitable means, an electric heater is shown. A suitably ceramic insulator 70 has a hollow central opening 71 large enough to pass the shaft 60 with proper clearance, has a shank portion 72 extending forward within the hollow of the drum and inside the electric heater 68, and has a flange portion 73 which extends outward against the flange 63 of the housing and is anchored to the housing by screws 74 extending into a mounting 75. The guidepost 37 is mounted in a screw 76 which extends into the mounting 75.

While it is preferred to provide the step 34 at the large end of the smooth descending conical portion of the drum as shown in my copending application above referred to, alternatively a step may be provided in the small end connecting the conical portion to a smooth cylindrical takeoff portion.

The drum is made of a heat-conducting metal, preferably aluminum. It is preferable also to use a coating on the outside of the drum to guard against staining the yarn, and this may be a cermet coating.

In operation of FIG. 1 two ends of synthetic continuous filament thermoplastic yarn are plied together so that each is twisted with respect to the other and then the plied ends are passed in one or more loops around the cylindrical pre-heating portion of the heater drum, passing around the guidepost as part of each loop. At the place where the most pronounced shrinkage takes place, the plied yarn falls over a step. Several loops of yarn are wrapped around a smooth descending conical portion, each of these loops passing around the guidepost. Then the yarn passes through the cooling device of the invention, being carried along as it is airborne under the streams of cooling gas. Finally, the yarn is separated or depiled and the individual bulked yarn ends having stretch characteristics are formed into packages.

On the heater drum an adjustment takes place brought about by backing up of twist from the point of separation of the bulked yarn ends to the heater drum, combined with the shrinkage effect, the adjustment being predominantly on the conical portion toward the takeoff end of the drum.

The preferred embodiment of the invention appears diagrammatically in FIG. 2, in which false twist imparts bulk to thermoplastic yarn by twisting the fibers to a predetermined number of twins per inch while the fibers are in softened condition due to the heat.

Yarn 20 from a source 21 passes through the hollow interior 76 of a false twist spindle 77 mounted on suitable bearings (not shown) and driven by a drive belt 78 travelling crosswise. The false twist spindle has a twisting head 80 provided with a pin 81 around which the yarn is wrapped. The yarn then passes to a takeup bobbin 82 on which the yarn is distributed by a traversing guide 83.

It will be evident that the pin 81 in the false twist head 80 provides a brake to the twist and that the false twist is applied upstream with respect to this head. Thus in a particular embodiment the number of turns of false twist applied while one inch of yarn is advancing may be 70 turns in a 70 denier yarn, and 90 turns in a 40 denier yarn, by way of example.

In the embodiment in FIG. 2 the false twist backs up to the yarn as it passes over the drum heater 30, which is suitably supplemented by a strip heater 42. The heater will raise the yarn into the thermoplastic range as described. Then the yarn will pass along the groove 46 of the cooling device 47, across the path of the jets of cooling gas 48. This cooling is applied to the still false twisted heated yarn and sets the twist, creating the memory condition which, once the yarn is downstream from the twist head, makes the yarn bulkier even though the twist is lost. It is important that the temperature be low enough after the yarn passes through the twist head so that little or no permanent twist will be removed. As the spindle speed increases, the number of wraps around the drum heater can be increased to allow enough time to heat properly to temperature. The rapid cooling necessary is imparted by the streams of gas in the cooling groove.

In some cases it is desirable to impart a forward or lifting component to the yarn as it is passing through the cooling groove. This is accomplished as shown in FIG. 7 by directing the orifice 48' diagonally forwardly so that they will impart a transverse component but also a forward or lifting component to the yarn as it progresses in the direction of the arrow 84. The form of FIG. 7 is preferred for vertical use of the cooling device.

In FIG. 8 I show a single step heater drum which may be used instead of the multistep drums of U.S. Pat. No. 3,420,983, above referred to, FIGS. 1, 3 and 4. The rotating drum 30' has a right cylindrical portion 33 at the inlet end 31, then an abrupt downward step 34, and then at the outlet end 32, it has a right cylindrical portion 84 which is divided by groove walls 85 into series yarn paths all of the same approximate diameter. The yarn passes around the separation pin 37 on each turn, passing from the inlet, over the step 34 and then, once it is heated to plastic temperature, through the grooves between the walls 85, in which false twist backs up before the yarn is cooled by the cooling means of the invention.

In view of my invention and disclosure, variations and modifications to meet individual whim or particular need will doubtless become evident to others skilled in the art, to obtain all or part of the benefits of my invention without copying the process and machine shown, and I therefore claim all such insofar as they fall within the reasonable spirit and scope of my claims.

Having thus described my invention that I claim as new and desire to secure by Letters Patent is:

1. In textile machinery, means for progressing synthetic thermoplastic continuous filament yarn forward, means for false twisting the yarn as it is progressed, a rotatably mounted heater drum having an inlet end receiving the yarn and a takeoff end directed toward the means for false twisting, the drum having an outside smooth cylindrical larger portion at the inlet end with which the yarn has contact, a smooth circular smaller portion toward the takeoff end from which the yarn leaves contact with the outside of the drum, and a downward step at one end of the smooth circular smaller portion, heater means inside the drum, a guide post beside the drum around which the yarn is wrapped for part of each turn, walls forming a cooling groove along which the yarn passes between the heater drum and the means for false twisting, means for progressing the yarn along the cooling groove and means for directing a plurality of streams of cooling gas into the groove against the yarn.

2. A machine of claim 1, in which the downward step is located at the large end of the circular smaller portion.

3. A machine of claim 1, in which the circular smaller portion is a descending conical portion.

4. A machine of claim 1, in which the circular smaller portion is a right cylinder.

5. In textile machinery, means for plying two ends of synthetic thermoplastic continuous filament yarn twisted with respect to one another, a rotatably mounted heater drum having an inlet end and a takeoff end, the drum having a smooth cylindrical larger portion which the yarn passes after leaving the heater drum, means for progressing the yarn along the cooling groove, orifice means distributed along the cooling groove for directing a plurality of streams of cooling gas into the groove at right angles to the direction of yarn progression, and means beyond the cooling groove for separating the two yarn ends to produce bulked yarn.

6. A machine of claim 5, in which the circular smaller portion is a descending cone.

7. A machine of claim 6, in which the downward step is located at the large end of the conical portion.

8. A machine of claim 5, in which the circular smaller portion is a right cylinder.

9. A process of bulking synthetic thermoplastic continuous filament yarn, which comprises twisting two ends of such yarn into plies, carrying the plied yarn around the outside of a smooth cylindrical larger portion of a rotatable heated drum and around a guide post in one or more loops, carrying the plied yarn around the outside of a smooth circular smaller portion of the heated drum and around the guide post in one or more loops, leading the yarn over an abrupt descending step at one end of the smooth conical portion, the temperature of heating of the yarn by the drum being within the thermoplastic range of the yarn, leading the plied yarn away from the drum adjacent to the small end of the conical portion, progressing the yarn along a groove, applying against the side of the yarn as it progresses along the groove a plurality of cooling gas streams, and separating the yarn ends to produce bulked yarn.

tion at the inlet end of which the plied yarn enters into contact with outside of the drum, a smooth circular smaller portion toward the takeoff end from which the plied yarn leaves contact with the outside of the drum, and a downward step at one end of the smooth circular smaller portion, heater means inside the drum, a guide post beside the drum around which the plied yarn is wrapped for part of each turn, walls forming a cooling groove along which the yarn passes after leaving the heater drum, means for progressing the yarn along the cooling groove, orifice means distributed along the cooling groove for directing a plurality of streams of cooling gas into the groove at right angles to the direction of yarn progression, and means beyond the cooling groove for separating the two yarn ends to produce bulked yarn.

6. A machine of claim 5, in which the circular smaller portion is a descending cone.

7. A machine of claim 6, in which the downward step is located at the large end of the conical portion.

8. A machine of claim 5, in which the circular smaller portion is a right cylinder.

9. A process of bulking synthetic thermoplastic continuous filament yarn, which comprises twisting two ends of such yarn into plies, carrying the plied yarn around the outside of a smooth cylindrical larger portion of a rotatable heated drum and around a guide post in one or more loops, carrying the plied yarn around the outside of a smooth circular smaller portion of the heated drum and around the guide post in one or more loops, leading the yarn over an abrupt descending step at one end of the smooth conical portion, the temperature of heating of the yarn by the drum being within the thermoplastic range of the yarn, leading the plied yarn away from the drum adjacent to the small end of the conical portion, progressing the yarn along a groove, applying against the side of the yarn as it progresses along the groove a plurality of cooling gas streams, and separating the yarn ends to produce bulked yarn.

\* \* \* \*